

## UNITED STATES PATENT OFFICE

2,354,088

## STABILIZED DIAZO-TYPE SENSITIVE MATERIAL

Maximilian K. Reichel, Albany, N. Y., assignor to  
General Aniline & Film Corporation, New York,  
N. Y., a corporation of Delaware

No Drawing. Application December 4, 1942.  
Serial No. 467,901

11 Claims. (Cl. 95—6)

This invention relates to the stabilization of light-sensitive layers which are produced by the incorporation of a diazo compound as the light-sensitive medium onto the surface of a suitable carrier base. More particularly, it refers to the stabilization of so-called dry development of two component diazo-type light-sensitive layers wherein the diazo compound is a diazo compound derived from ortho or para aminonaphthol or from N-mono or di-substituted aromatic para-diamines such as para amino aniline compounds, which diazo compound is incorporated into the light-sensitive layer, together with an azo dyestuff coupling component.

Various processes are known for the preparation of light-sensitive layers which depend upon the use of a diazo compound as the light-sensitive medium, and various materials have been employed for the carrier of the light-sensitive layer, including textiles, paper, cellulosic films, and glass and metal surfaces. The sensitized carrier is exposed to light under a transparent original which it is desired to reproduce and the diazo compound is decomposed in the areas unprotected by the outline of the original. The undecomposed diazo compound in the protected areas is then used to develop the image of the original by coupling the said diazo compound in alkaline atmosphere with an azo dyestuff coupling component. In the two component layers which contemplate the incorporation of the coupling component into the light-sensitive layer with the diazo compound, the development of the dyestuff forming the image is effected by bringing the exposed light-sensitive layer into contact with ammonia gas. This is known as the dry developing process.

The dyestuff components, as applied on the carrier, are relatively unstable and cannot be stored for long periods prior to use.

The light-sensitive layers which carry the coupling component as well as the diazo compound in the light-sensitive layer are subject to premature coupling of the said dyestuff components as well as decomposition of the diazo compound upon long storage. Many attempts have been made to obtain more stable coating solutions and to render the light-sensitive layers produced therefrom less sensitive to deterioration without impairing the light-sensitive qualities of the diazo compound upon which the production of accurate images from the original depends. These attempts have hitherto been relatively unsuccessful. It is therefore the object of this invention to provide coating solutions and light-sensitive

layers, using diazo compounds as the light-sensitive medium which can be stored for long periods prior to use and will be stable during storage even under unfavorable conditions.

I have found that coating solutions and the light-sensitive layers prepared therefrom can be stabilized against decomposition of the light-sensitive material and premature coupling of the dyestuff components by adding to the coating solution a compound of the following class: alpha-beta unsaturated acrylic acids and the alkali metal salts thereof having the general formula:



Wherein R stands for a radical of the group consisting of alkyl, phenyl, pyridyl, quinolyl, and substituted phenyl, pyridyl and quinolyl radicals. Examples of such compounds are:

Crotonic acid



Pentene acid



Sulfo-cinnamic acid



Beta(alpha-pyridyl)-acrylic acid



Beta-2-methyl-quinolyl (5)-acrylic acid



The compounds of this group can exist in both the cis- and trans- form, either of which is suitable for the purposes of this invention. Diazo-type light-sensitive layers which have been stabilized by addition of compounds selected from the above group show greatly improved keeping qualities and are stable against decomposition or deterioration for much longer periods of storage than has been possible with the same diazo light-sensitive compositions lacking this stabilizing

compound or in which previously suggested stabilizing compounds have been used. The following examples illustrate the invention but they are not intended to limit it thereto. The parts are by weight unless otherwise stated.

**Example I**

2-1-diazo-hydroxy-naphthalene- $\alpha$ -sulfonic acid parts 14.0

Conc. hydrochloric acid parts by volume 7.0

Nickel sulphate parts 21.5

Phloroglucine do 4.9

Thiourea parts 20.0

were dissolved in 1000 cc. of water. Before coating there were added 8.74 grams per liter of crotonic acid. This solution was then spread on paper, fabric, film or the like by the usual coating method, using a doctor blade to insure a thin even coating. After storage at room temperature for several months, the stability of the sensitized material containing the crotonic acid was tested by exposing a test piece to light under a suitable diapositive and developing the image by application of ammonia gas. The resulting image reproduced on the light-sensitive layer containing the crotonic acid was compared with the image reproduced under the same conditions on a light-sensitive layer made from the same materials but containing no crotonic acid which had been stored under the same conditions for the same length of time. The background and consequently the contrast of the image reproduced on the light-sensitive layer made in accordance with this example was superior to that of the sample which does not contain the crotonic acid in the light-sensitive layer.

**Example II**

The procedure is the same as in Example I except that in place of the crotonic acid as a stabilizer 10.0 grams of pentene acid per liter are used. The stability of the coating made according to this example was found to be superior to that of a comparison coating made from a similar coating solution but containing no acrylic acid stabilizer.

**Example III**

The procedure is the same as in Example I except that in place of the crotonic acid as stabilizer 25.5 grams of sulfo-cinnamic acid per liter is used. The stability of the coating made according to this example was found to be superior to that of a comparison coating made from a similar coating solution but containing no acrylic acid stabilizer.

**Example IV**

The composition of the coating solution is the same as in Example I except that in place of the crotonic acid as a stabilizer, 15.15 grams of beta(alpha-pyridyl)-acrylic acid per liter are employed. To facilitate solution 50 cc. of alcohol are added to the water. The stability of the coating made according to this example was found to be superior to that of a comparison coating made from a similar coating solution but containing no acrylic acid stabilizer.

**Example V**

The procedure is the same as in Example I except that in place of the crotonic acid as a stabilizer 21.6 grams of beta-(2-methyl-quinuclidyl)-(5)-acrylic acid are used. To facilitate solution

50 cc. of isopropanol are added. The stability of the coating made according to this example was found to be superior to that of a comparison coating made from a similar coating solution but containing no acrylic acid stabilizer.

**Example VI**

Parts

Zinc chloride double salt of the diazo-com-  
pound obtained from N-ethanol-ethyl  
amino-4-aminobenzene 10.5

Citric acid 50

2-3-dihydroxy-naphthalene 5.0

Thiourea 45

The sodium salt of the naphthalene-1-3-6-trisulfonic acid 32.5

Aluminum sulphate 6.9

were dissolved in 1000 cc. of water. Before coating there were added 25.5 grams of sulfo-cinnamic acid. This solution was spread on a suitable base, such as paper, fabric, film or the like, by the usual coating method in the same manner as indicated in Example I. The light-sensitive layer thus produced was then stored at room temperature for several months and its stability then tested by observing the appearance of color in the light-sensitive layer due to premature coupling of the dye components and by comparison of its light-sensitive qualities with those of a test sample prepared and treated in the same manner as the light-sensitive layer of this example but omitting the sulfo-cinnamic acid addition. It was found that the light-sensitive layers made in accordance with this example show a negligible amount of coloring due to premature coupling of the dye components, whereas light-sensitive layers made from the same solution, but not having the stabilizing agent, which have been stored under the same conditions for the same length of time, show a considerable amount of coloring due to premature coupling. It was also found that upon exposure to light under a suitable diapositive and development of the image by application of ammonia gas, the light-sensitive layers of this example produce images having better contrast due to less background color than do light-sensitive layers not having the stabilizing agent, but otherwise having been made and treated the same as the light-sensitive layers of this example.

**Example VII**

The procedure is the same as in Example VI except that in place of sulfo-cinnamic acid as a stabilizer 8.74 grams of crotonic acid per liter are used. The stability of the coating made according to this example was found to be superior to that of a comparison coating made from a similar coating solution but containing no acrylic acid stabilizer.

**Example VIII**

The procedure is the same as in Example VI except that in place of sulfo-cinnamic acid as a stabilizer 10.0 grams of pentene acid per liter are used. The stability of the coating made according to this example was found to be superior to that of a comparison coating made from a similar coating solution but containing no acrylic acid stabilizer.

**Example IX**

The procedure is the same as in Example VI except that in place of sulfo-cinnamic acid as a stabilizer, 15.15 grams of beta(alpha-pyridyl)-acrylic acid per liter are used. To facilitate solu-

tion 50 cc. of alcohol are added. The stability of the coating made according to this example was found to be superior to that of a comparison coating made from a similar coating solution but containing no acrylic acid stabilizer.

*Example X*

The composition of the coating solution is the same as in Example VI, except that in place of sulfo-cinnamic acid as a stabilizer, 21.6 grams of beta-2-methyl-quinolyl (5)-acrylic acid are used. To facilitate solution 50 cc. of isopropanol are added. The stability of the coating made according to this example was found to be superior to that of a comparison coating made from a similar coating solution but containing no acrylic acid stabilizer.

*Example XI*

|                                                                                                              | Parts |
|--------------------------------------------------------------------------------------------------------------|-------|
| Zinc chloride double salt of the diazo compound obtained from N-monoethyl-amino 2 methyl 4 aminobenzene----- | 9.8   |
| Citric acid-----                                                                                             | 50    |
| Resorcine-----                                                                                               | 6.5   |
| Thiourea-----                                                                                                | 45    |
| The sodium salt of the naphthalene-1,3,6, trisulfonic acid-----                                              | 32.5  |
| Aluminum sulfate are dissolved in 1000 cc. of water-----                                                     | 6.9   |

To this solution there are added 25.5 grams of sulfo-cinnamic acid per liter. The coating, storage and testing procedures are the same as in Example I. The stability of the coating made according to this example was found to be superior to that of a coating made from a solution not containing an acrylic acid stabilizer.

*Example XII*

|                                                                                                          | Parts |
|----------------------------------------------------------------------------------------------------------|-------|
| Zinc chloride double salt of the diazo compound obtained from N-ethanol-ethyl-amino 4 amino-benzene----- | 10.5  |
| Citric acid-----                                                                                         | 5     |
| Thiourea-----                                                                                            | 45    |
| The sodium salt of the naphthalene-1,3,6, trisulfonic acid-----                                          | 32.5  |
| Aluminum sulfate are dissolved in 1000 cc. of water-----                                                 | 6.9   |

To this solution there are added 25.5 grams of sulfo-cinnamic acid per liter. The solution is then spread on a suitable base, such as paper, fabric, film or the like by the usual coating method in the same manner as described in Example I. The light-sensitive layer thus produced is then stored at room temperature for several months, and its stability is then tested by observing the appearance of color in the light-sensitive layer due to decomposition of the diazo-compound and by comparison with that of a test sample prepared and treated in the same manner as the light-sensitive layer of this example but omitting the sulfo-cinnamic acid. The test pieces are then exposed to light under a suitable diapositive and the images developed by application of an alkali solution of a suitable azo component such as phloroglucine, resorcine, or 2-3-dihydroxy-naphthalene. The resulting image produced on the light-sensitive layer containing the sulfo-cinnamic acid showed a much higher color contrast of the images indicating the prevention of the decomposition and the consequent discoloration of the diazo-compound while at storage under the same length of time.

Various changes may be made in the details of my invention as described in the foregoing spec-

ification within the scope of the claims appended hereto without sacrificing the advantages of my invention.

I claim:

1. The process of increasing the stability of a diazotype light-sensitive layer containing a suitable diazo compound which comprises adding to the coating solution an alpha-beta-unsaturated acrylic acid of the following formula:



wherein R stands for a radical selected from the group consisting of alkyl, phenyl, pyridyl, quinolyl and substituted phenyl, pyridyl and quinolyl radicals, and coating a suitable base with said solution.

2. The process of increasing the stability of a diazotype light-sensitive layer containing a diazo compound suitable for forming a stable two component diazotype layer and an azo dye coupling component, which comprises adding to the coating solution an alpha-beta-unsaturated acrylic acid of the following formula:



wherein R stands for a radical selected from the group consisting of alkyl, phenyl, pyridyl, quinolyl and substituted phenyl, pyridyl and quinolyl radicals, and coating a suitable base with said solution.

3. The process of increasing the stability of a diazotype light-sensitive layer containing a diazo compound derived from a para amino aniline compound and an azo dye coupling component, which comprises adding to the coating solution containing the said diazo compound an alpha-beta-unsaturated acrylic acid of the following formula:



wherein R stands for a radical selected from the group consisting of alkyl, phenyl, pyridyl, quinolyl and substituted phenyl, pyridyl and quinolyl radicals, and coating a suitable base with said solution.

4. The process of increasing the stability of a diazotype light-sensitive layer containing a diazo compound obtained from an ortho amino naphthol compound and an azo dye coupling component, which comprises adding crotonic acid to the coating solution and coating a suitable base with said solution.

5. The process of increasing the stability of a diazotype light-sensitive layer containing a diazo compound obtained from a para amino aniline compound and an azo dye coupling component, which comprises adding sulfo-cinnamic acid to the coating solution and coating a suitable base with said solution.

6. The process of increasing the stability of a diazotype light-sensitive layer containing a diazo compound obtained from a para amino aniline compound and an azo dye coupling component, which comprises adding pentene acid to the coating solution and coating a suitable base with said solution.

7. Light-sensitive layers on a suitable base comprising a diazo compound suitable for forming a stable two component diazotype layer, an azo

dyestuff coupling component and an alpha-beta-unsaturated acrylic acid of the following formula:



wherein R stands for a radical selected from the group consisting of alkyl, phenyl, pyridyl, quinolyl and substituted phenyl, pyridyl and quinolyl radicals.

8. Light-sensitive layers on a suitable base comprising a diazo compound obtained from a para amino aniline compound, an azo dye coupling component, and an alpha-beta-unsaturated acrylic acid of the following formula:



wherein R stands for a radical selected from the group consisting of alkyl, phenyl, pyridyl, quinolyl and substituted phenyl, pyridyl and quinolyl radicals.

9. Light-sensitive layers on a suitable base comprising a diazo compound obtained from an ortho amino naphthol compound, an azo dye coupling component and crotonic acid.

10. Light-sensitive layers on a suitable base comprising a diazo compound obtained from a para amino aniline compound, an azo dye coupling component and sulfo-cinnamic acid.

11. Light-sensitive layers on a suitable base comprising a diazo compound obtained from a para amino aniline compound, an azo dye coupling component and pentenic acid.

MAXIMILIAN K. REICHEL.